

Aug. 20, 1963

L. H. MESSINGER

3,100,925

APPARATUS FOR COMPRESSIVE FINISHING OF FABRICS

Filed Dec. 2, 1960

**FIG. 1**



1

3,100,925

APPARATUS FOR COMPRESSIONAL FINISHING  
OF FABRICS

Lester Hubert Messinger, Newark, Del., assignor to E. I. du Pont de Nemours and Company, Wilmington, Del., a corporation of Delaware

Filed Dec. 2, 1960, Ser. No. 73,433  
3 Claims. (Cl. 26—18.6)

This invention relates generally to the production of fabrics, and more particularly to novel process and apparatus improvements in the finishing of fabrics, especially those fabrics which are constructed from a preponderance of man-made filamentary material and to treatment to control and stabilize residual shrinkage within acceptable limits.

Conventional methods of finishing fabrics in the past have involved the use of apparatus designed to handle the natural fibers, such as those made of wool, cotton, and the like. These conventional finishing methods have been carried out on fabrics under conditions such that the fabrics are, during most of the finishing treatments, under varying degrees of tension. Recently, a new machine has been developed whereby the fabric is compressed or compacted in the warp direction by means of two rolls rotating at different speeds and a doctor blade tangentially located with respect to the faster moving roll. In this treatment of fabric all the compressional work is done in a short space between the nip of the doctor blade with the faster moving roll and the nip of the two rolls, which leads to relatively minor fabric improvements. However, this improvement is of value since the prior treatments of fabric under tension always led to changes in dimensions (shrinkage) of the fabric while in use due to the gradual relief of these tensions in home or commercial laundries.

The principal object of this invention is to provide an improved process and apparatus suitable for finishing all types of fabrics, woven and non-woven, and particularly synthetic fabrics, while held under compression. Another object is the processing of such fabrics through such well-known wet finishing steps as scouring, heat setting, dyeing, and the like in a manner such that the finished fabric is substantially free from internal tensions and is stabilized to a superior degree when compared to prior finishing techniques, as to further changes in dimensions during use of the fabric. Another object is to reduce the pucker accompanying the seam sewing of fabrics made particularly of man-made filamentary materials. Other objects and advantages will be apparent from the following description of the invention, the drawings, and the accompanying claims.

The above objects are accomplished by an improved apparatus embodying features of the present invention, which generally comprises means for continuously feeding a fabric, which is supported discontinuously at a plurality of points, to a card clothing belt having projections protruding above the surface thereof, while passing superheated steam through the fabric held under compression. Preferably, the fabric is conducted over the surface of a foraminous metal drum, through which steam passes to permeate the fabric. The invention also comprises apparatus for wet-finishing of fabrics which will be more fully described below by reference to the accompanying drawings in which:

FIGURE 1 is a perspective partly schematic view of a machine embodying features of this invention, with certain parts broken away.

FIGURE 2 is an enlarged side view of the card clothing belt showing its construction with the wire staples.

FIGURE 3 is a somewhat enlarged end view of the

2

main rollers and card clothing belt engaging the fabric, illustrating the compacting action of the staples on the fabric.

FIGURE 4 is an oblique view of an alternative roll configuration to be used when it is desired to achieve fabric compaction simultaneously in transverse and longitudinal directions.

Referring to the drawings, the fabric 1 is fed from roll 2, shown in FIGURE 1, to a pair of resilient pinch rolls 3 and 4, made of rubber or other suitable material, which meter the fabric 1 to a bite between shield 5 and endless belt 6 shown enlarged in FIGURE 2. This belt is made up of card clothing such as is used in normal carding equipment and consists essentially of wire staples 30 driven through a canvas and rubber belt 31. There are approximately 670 projecting wires in one square inch of this belting. At the point where the fabric 1 enters the bite between the shield 5 and belt 6, the back 31 of the belt 6 is against roll 7 and the ends of the wires 30 are spread apart (zone b, FIGURE 3) or divergent with respect to the direction of belt movement due to the flexing of the belt as it conforms to the radius of curvature of the roll 7. The shield 5 holds the fabric 1 against the belt 6 until it transfers from roll 7 to roll 8. As the belt 6 reverses its curvature, the wires 30 are now between the canvas rubber backing 31 and the roll 8, and this causes the wires to converge toward the free ends thereof and the longitudinal spacings between the free ends of the wires 30 are greatly reduced (zone c, FIGURE 3), resulting in longitudinal compression or compaction of the fabric. Simultaneous transverse and longitudinal compaction may be achieved by utilizing roll configurations as illustrated in FIGURE 4 for rolls 7 and 8 or roll 7 alone. Roll 8 is a foraminous construction, preferably made of porous metal or provided with passages 80 and is connected, to a steam line by suitable means such as a hollow drive shaft 81. Steam is introduced into the interior of roll 8 so that a definite steam pressure is maintained therein. Steam flows through the foraminous walls of roll 8 and blows directly through the fabric before losing its throttling superheat. Belt 6 holds the fabric 1 on the steam roll 8 until the belt is taken off the fabric by roll 9. The fabric 1 continues in contact with the steam roll 8 until after it passes under roll 10, when it is lifted off and wound up without appreciable tension by contact with rubber roll 11. The machine is driven by the chain 41 at sprockets 44, 43, and 42. V-belt pulleys 47 and 48 are adjustable in a conventional manner to control fabric hold-back. Roll 9 is driven faster than rolls 7 and 13 through slip clutch 49 in order that the fabric pressure on the steam roll 8 may be adjusted by varying the slip torque of the clutch. The wind-up roll 11 is driven by the V-belt on pulleys 45 and 46. Using a six-inch diameter for rolls 7 and 8, a warp-wise compression or compaction in the fabric of approximately 36% has been obtained.

As one illustration of the process aspects of this invention, a suiting fabric produced from spun yarns composed of 80% acrylonitrile polymer fiber and 20% wool and treated on the above-described apparatus, achieved a total reduction in length of the fabric of 18%. This contrasted with a 6% reduction in length obtained when the same fabric, untreated by the arrangement of this invention, was vigorously steamed at atmospheric pressure for five minutes. The fabric treated on this apparatus had excellent stability to subsequent washing and scouring operations, and had markedly improved cover and fullness.

The process of this invention may be applied to improve the properties of many types of fabrics such as woven, knitted, and non-woven fabrics. The fabrics may be com-

posed of any synthetic or natural staple fibers and/or continuous filaments. Typical examples of man-made filamentary materials include those made from polyamides such as poly(hexamethylene adipamide), poly(hexamethylene sebacamide), polycaproamide and copolyamides; polyesters and copolyesters, such as condensation products of ethylene glycol with terephthalic acid, ethylene glycol with a 90/10 mixture of terephthalic and isophthalic acids, ethylene glycol with a 98/2 mixture of terephthalic and 5-(sodium sulfo)-isophthalic acids, and trans-p-hexahydroxyethylene glycol with terephthalic acid; polyacrylonitrile, copolymers of acrylonitrile with other monomers such as vinyl acetate, vinyl chloride, methyl acrylate, vinyl pyridine and sodium styrene sulfonate, terpolymers of acrylonitrile, methyl acrylate and sodium styrenesulfonate made in accordance with U.S. Patent 2,837,501; vinyl and vinylidene polymers and copolymers, polycarbonates, polyurethanes, polyesteramides, polyethylenes, polypropylenes, fluorinated ethylene polymers and copolymers; composite filaments such as, for example, a sheath of polyamide around a core of polyester as described in the copending application of Breen, S.N. 621,443, filed November 9, 1956, now abandoned, and two acrylonitrile polymers differing in ionizable group content spun as a sheath and core as described in the copending application of Taylor, S.N. 771,677, filed November 3, 1958, now U.S. Patent S.N. 3,038,237, and the like. Examples of cellulose derivative fibers include cellulose acetate, cellulose triacetate and regenerated cellulose. The natural fibers include cotton, wool, silk and the like. The fibers and filaments may be crimped or uncrimped, drawn or undrawn, and/or bulked or unbalked. Two or more fibers or filaments may be blended together in making the fabrics to be processed. Particularly, improved results are obtained when applying the treatment of this invention to fabrics composed either entirely of man-made filamentary material or of a blend of at least 50% man-made filamentary material combined with lesser amounts of natural fibers and/or cellulose derivative fibers.

The chief advantage of this invention is that it provides a process and apparatus for the wet finishing of fabrics which results in fabrics that are preshrunk and are much more stable to use and laundering than the same fabrics finished by prior methods. In addition, the resulting fabrics finished by this invention are more resilient and elastic which causes less pucker in seam sewing the fabrics, they have a more pleasing hand that is more comfortable to the wearer, they possess less wrinkling, bagging, massing, fuzzing, and they exhibit improved crease and shape retention, when compared to the same fabrics finished by conventional means. Another advantage of this invention is that it relieves the tension normally present in commercially finished fabrics without the usual flattening of the fabrics so that they resist changes in dimensions on subsequent washing. The present invention also permits liquids and gases such as steam to be forced through the fabric while it is being compressed or compacted. The treatment of this invention achieves best results on heavy fabrics not tightly constructed.

The process and apparatus of this invention, being capable of continuous use, may be used for finishing fabrics either alone or more advantageously in conjunction with other types of finishing treatments, such as calendering, napping, shearing, heat setting, a scouring, dyeing, and the like.

Another illustration of the process aspects of this invention, as well as its utility and advantages is given by the following example:

#### Example

This example illustrates the treatment of a woven fabric made from yarn which was a blend of 18.5% by weight of 6 denier polyester staple fiber, 36.5% by weight of 3 denier polyester staple fiber, and 45% of 70's wool. The polyester fiber used was polyethylene terephthalate. The

woven fabric was napped in the griee with two passes on the face and one pass on the back on a Gessner Rotary Napper, cropped on a Curtis-Marble single-blade shear, beck scoured at the boil for 1 hour and then dried. At this point, the fabric was cut into two equal pieces and each piece was given a different finishing treatment. Sample A was finished on the special apparatus pictured in FIGURE 1 and sample B was given a conventional wet finishing treatment.

After each of the fabrics was subjected to the respective finishing treatments, both fabrics were given the same final finishing treatment, as follows:

- (1) Napped—face only on a Gessner Rotary Napper.
- (2) Brushed and sheared—on a Curtis-Marble single-blade shear.
- (3) Heat set—at 330° F. for 1 minute exposure, dry width, with 4% overfeed in filling direction.
- (4) Rotary pressed—at 300° F.
- (5) Semidecated—for 3 minutes with steam and 1 minute with vacuum.

Each of the two sample fabrics was subjected to certain tests for measurement of fabric properties, and the results given in Table I show the superior properties of those fabrics finished by this invention in comparison with conventionally finished fabrics.

It has been found that particularly desirable results are obtained when fabrics are first subjected to the compressional treatment of this invention, followed by the impact oscillatory treatment described in my copending application U.S. Ser. No. 5,528, filed January 29, 1960, now U.S. Patent No. 3,064,459. This sequence of treatments for a fabric greatly improves the stability of the fabric to resist changes in shape and dimensions during conventional washing, laundering and drying cycles.

Table I

| Sample | Hours' wear | Wrinkle | Crease retention | Bagging | Mussiness | Fuzzing |
|--------|-------------|---------|------------------|---------|-----------|---------|
| A----- | 100         | 2.5     | 2.1              | 1.9     | 2.0       | 1.3     |
|        | 250         | 2.9     | 2.6              | 2.2     | 2.1       | 1.6     |
|        | 450         | 2.9     | 2.8              | 2.6     | 2.8       | 1.9     |
|        | 550         | 2.9     | 2.9              | 2.3     | 2.4       | 1.9     |
|        | 100         | 2.8     | 2.7              | 2.0     | 2.3       | 2.1     |
| B----- | 250         | 2.6     | 2.9              | 2.6     | 2.5       | 2.0     |
|        | 450         | 3.6     | 3.4              | 2.7     | 3.2       | 2.0     |
|        | 550         | 3.7     | 3.3              | 2.5     | 2.4       | 2.1     |
|        |             |         |                  |         |           |         |

NOTE.—1, no change from original; 2, slight change from original; 3, borderline objectionable; 4, objectionable; 5, unwearable.

These figures indicate that the sample A fabrics were superior to the sample B conventionally finished fabrics since they did not exceed the rating borderline objectionable in any test.

In accordance with the patent statutes, I have set forth a detailed description of preferred embodiments of my invention. It will be obvious that modifications and other embodiments may be made by those skilled in the art without departing from the spirit of the invention or the scope of the following claims:

I claim:

1. An improved apparatus for treatment of a fabric to increase its resistance to shrinkage, its cover, and its fullness, comprising in combination, a first means for continuously moving a fabric having a given width and a given thickness from a first location to a second location, a second means positioned between the first and second locations engaging the fabric evenly throughout its thickness at a substantially uniformly distributed plurality of points in a first zone, a third means cooperating with said second means to apply a sufficient force through said second means to said fabric at each of said points in said first zone and evenly throughout the thickness of the fabric in a direction in the plane of the fabric such that the spacing between said points is reduced and the thickness of the fabric is increased without pleating to produce a compression and compaction of the fabric in at least one direction,

a fourth means for maintaining elevated conditions of temperature and humidity in said zone during application of said force to said fabric, a fifth means cooperating with said third means to terminate application of said force to said fabric, a sixth means for releasing engagement of said second means with said fabric, in which said second means comprises an endless belt, said belt provided with an operative surface in which are secured a plurality of evenly distributed flexibly-mounted projecting fabric-penetrating elements, each having a fabric penetrating end and supported to move in a path which converges with the path of movement of said fabric in said first zone and causes engagement of said elements with said fabric at said plurality of points, in which said third means comprises an element with a cylindrical surface in engagement with said endless belt to change the direction of movement thereof in a curved path such that the flexibly-mounted elements converge to move the fabric-penetrating ends towards each other and compress the fabric surrounding said flexibly-mounted elements, in which said fourth means comprises a steam chamber located in said element with the cylindrical surface and a plurality of steam escape passages connecting said chamber with said cylindrical surface.

2. An improved machine for continuous treatment of a fabric to increase its resistance to shrinkage and enhance its cover and fullness characteristics comprising in combination, a supporting frame structure, drive means mounted in said structure to engage and move a running length of fabric through a given path from a starting position to a final position, a fabric compaction and heat treating assembly mounted in said structure in operative association with said given path of fabric movement, said assembly comprising an endless belt member mounted in said frame structure for movement through a path of movement a portion of which at a given location substantially coincides with a portion of the given path of movement of said fabric length, a drive means for said belt member, said belt member comprising a backing element and a plurality of elongated flexibly-mounted elements, projecting from one surface thereof, said flexibly-mounted elements being of substantially equal length and each provided with a fabric-penetrating portion at the projecting end thereof, said belt member so positioned and moved with respect to said fabric that as said belt member approaches said fabric at the location of substantial coincidence of their paths of movement, said flexibly-mounted elements penetrate said fabric to positively engage it evenly throughout its thickness at a plurality of points, said assembly further comprising an elongated cylindrical element mounted transversely to the direction of fabric and belt movement in said supporting frame structure and in engagement with said belt member in said given location of coinciding paths of said fabric and belt member to deflect and guide the belt member in a curved path such that the side of said belt member carrying said flexibly-mounted projecting elements moves through a concavely curved path so that the spacing between said ends of said flexibly-mounted elements is decreased due to flexing of the belt member on which the elements are mounted by

5

15

20

25

30

35

40

45

50

55

60

the action of said elongated cylindrical element, which decrease in spacing causes a continuous compaction and increase in thickness of said moving fabric engaged by said fabric penetrating portions of said flexibly-mounted elements in said given location, said elongated cylindrical element comprising an exterior surface, an interior chamber, an inlet for the reception of steam under pressure, and a substantially evenly distributed plurality of small steam escape passages connecting said interior chamber with said exterior surface to direct escaping steam on the fabric engaged by the penetrating portions of the flexibly-mounted elements of the belt member as such belt member is being deflected and guided by said elongated cylindrical element.

3. An improved apparatus for treatment of a fabric to increase its resistance to shrinkage, its cover, and its fullness, comprising in combination, a first means for continuously longitudinally moving a fabric having a given width and a given thickness from a first location to a second location, a second means positioned between the first and second locations engaging the fabric evenly throughout its thickness at a substantially uniformly distributed plurality of points in a first zone, a third means cooperating with said second means to apply a sufficient force through said second means to said fabric at each of said points in said first zone and evenly throughout the thickness of the fabric in a direction in the plane of the fabric such that the spacing between said points is reduced and the thickness of the fabric is increased without pleating to produce a compression and compaction of the fabric simultaneously in the direction of its width and longitudinally, a fourth means for maintaining elevated conditions of temperature and humidity in said zone during application of said force to said fabric, in which said second means comprises an endless belt, said belt provided with an operative surface in which are secured a plurality of evenly distributed flexibly-mounted projecting fabric-penetrating elements, each having a fabric penetrating end and supported to move in a path which converges with the path of movement of said fabric in said first zone and causes engagement of said elements with said fabric at said plurality of points, in which said third means comprises an element with a cylindrical surface in engagement with said endless belt to change the direction of movement thereof in a curved path such that the flexibly-mounted elements converge to move the fabric-penetrating ends towards each other and compress the fabric surrounding said flexibly-mounted elements, in which said fourth means comprises a steam chamber located in said element with the cylindrical surface and a plurality of steam escape passages connecting said chamber with said cylindrical surface.

References Cited in the file of this patent

UNITED STATES PATENTS

2,120,536 Woodhead ----- June 14, 1938  
2,535,734 Grettve ----- Dec. 26, 1950

FOREIGN PATENTS

453,187 Great Britain ----- Sept. 7, 1936